



US007473284B2

(12) **United States Patent**  
**Krull**

(10) **Patent No.:** **US 7,473,284 B2**  
(b4) **Date of Patent:** **\*Jan. 6, 2009**

(54) **FUEL OILS COMPOSED OF MIDDLE DISTILLATES AND OILS OF VEGETABLE OR ANIMAL ORIGIN AND HAVING IMPROVED COLD FLOW PROPERTIES**

6,409,778 B1 6/2002 Auschra  
6,458,175 B1 10/2002 Tack  
6,461,393 B1 10/2002 Krull  
6,509,424 B1 1/2003 Krull

(75) Inventor: **Matthias Krull**, Harxheim (DE)

(Continued)

(73) Assignee: **Clariant Produkte (Deutschland) GmbH**, Sulzbach (DE)

## FOREIGN PATENT DOCUMENTS

(\*) Notice: Subject to any disclaimer, the term of this patent is extended or adjusted under 35 U.S.C. 154(b) by 835 days.

This patent is subject to a terminal disclaimer.

CA 2008986 8/1990  
CA 2017126 11/1990  
CA 2020104 12/1990  
CA 2055417 5/1992  
DE 3443 475 5/1986  
DE 4134347 4/1993  
EP 0203 554 12/1986  
EP 0254 284 1/1988  
EP 0271 738 6/1988  
EP 0 308 176 3/1989

(21) Appl. No.: **10/972,577**

(Continued)

(22) Filed: **Oct. 25, 2004**

(65) **Prior Publication Data**

US 2005/0126070 A1 Jun. 16, 2005

## OTHER PUBLICATIONS

German Patent Office—Office Action for DE 103 57 878.1, Apr. 26, 2006.

(30) **Foreign Application Priority Data**

Dec. 11, 2003 (DE) 103 57 878

(Continued)

(51) **Int. Cl.**

**C10L 1/18** (2006.01)

*Primary Examiner*—Cephia D Toomer

(74) *Attorney, Agent, or Firm*—Richard P. Silverman

(52) **U.S. Cl.** 44/393; 44/395; 44/397

(57) **ABSTRACT**

(58) **Field of Classification Search** 44/393, 44/395, 397

The invention provides a fuel oil composition F) comprising F1) a fuel oil of mineral origin and

See application file for complete search history.

F2) a fuel oil of vegetable and/or animal origin, and, as a cold additive, the constituents

(56) **References Cited**

A) at least one copolymer composed of ethylene and 8-21 mol % of at least one acrylic or vinyl ester having a C<sub>1</sub>-C<sub>18</sub>-alkyl radical and

## U.S. PATENT DOCUMENTS

B) at least one comb polymer containing structural units having C<sub>8</sub>-C<sub>16</sub>-alkyl radicals, the structural units being selected from C<sub>8</sub>-C<sub>16</sub>-alkyl (meth)acrylates, C<sub>8</sub>-C<sub>16</sub>-alkyl vinyl esters, C<sub>8</sub>-C<sub>16</sub>-alkyl vinyl ethers, C<sub>8</sub>-C<sub>16</sub>-alkyl(meth) acrylamides, C<sub>8</sub>-C<sub>16</sub>-alkyl allyl ethers and C<sub>8</sub>-C<sub>16</sub>-diketenes,

where the sum R

3,462,249 A 8/1969 Tunkel  
4,211,534 A 7/1980 Feldman  
4,608,411 A 8/1986 Meunier  
4,670,516 A 6/1987 Sackmann  
4,713,088 A 12/1987 Tack  
4,810,260 A 3/1989 Tack  
4,906,682 A 3/1990 Mueller  
5,017,299 A 5/1991 Gutierrez  
5,045,088 A 9/1991 More  
5,178,641 A 1/1993 Konrad  
5,186,720 A 2/1993 Feustel  
5,200,484 A 4/1993 Reimann  
5,254,652 A 10/1993 Feustel  
5,275,747 A 1/1994 Gutierrez  
5,391,632 A 2/1995 Krull  
5,413,725 A 5/1995 Lal  
5,439,981 A 8/1995 Reimann  
5,441,545 A 8/1995 Lewtas  
5,733,346 A 3/1998 Davies  
5,743,923 A 4/1998 Davies  
5,767,190 A 6/1998 Krull  
5,789,510 A 8/1998 Krull  
5,833,722 A 11/1998 Davies  
5,858,028 A 1/1999 Davies  
6,086,645 A 7/2000 Quigley  
6,162,772 A 12/2000 Panagiotis  
6,232,277 B1 5/2001 Ledeore  
6,306,186 B1 10/2001 Davies  
6,384,170 B1 5/2002 Krull

of the molar averages of the carbon chain length distributions in the alkyl radicals of the monomers B) is from 11.0 to 14.0, where

m<sub>1</sub>, m<sub>2</sub>, ..., m<sub>g</sub> are the molar fractions of the abovementioned monomers B) in the polymer, and the sum of the molar fractions m<sub>1</sub> to m<sub>g</sub>=1,  
w<sub>1i</sub>, w<sub>1j</sub> ..., w<sub>2i</sub>, w<sub>2j</sub> ..., w<sub>gp</sub> are the proportions by weight of the individual chain lengths i, j, p of the alkyl radicals of the different monomers B) 1 to g, and

n<sub>1i</sub>, n<sub>1j</sub> ..., n<sub>2i</sub>, n<sub>2j</sub> ..., n<sub>gp</sub> are the chain lengths of the alkyl radicals i, j, ..., p of the monomers B) 1 to g.

20 Claims, No Drawings

## U.S. PATENT DOCUMENTS

|                 |         |          |
|-----------------|---------|----------|
| 6,565,616 B1    | 5/2003  | Krull    |
| 6,592,638 B2    | 7/2003  | Krull    |
| 6,638,325 B1    | 10/2003 | Brod     |
| 2001/0034308 A1 | 10/2001 | Krull    |
| 2001/0034410 A1 | 10/2001 | Krull    |
| 2002/0099228 A1 | 7/2002  | Krull    |
| 2003/0119992 A1 | 6/2003  | Deneker  |
| 2003/0136046 A1 | 7/2003  | Jackson  |
| 2004/0006912 A1 | 1/2004  | Krull    |
| 2005/0108924 A1 | 5/2005  | Krull    |
| 2005/0113266 A1 | 5/2005  | Krull    |
| 2005/0126071 A1 | 6/2005  | Krull    |
| 2005/0126072 A1 | 6/2005  | Krull    |
| 2006/0137242 A1 | 6/2006  | Siggekow |
| 2007/0157509 A1 | 7/2007  | Siggekow |
| 2007/0161755 A1 | 7/2007  | Siggekow |

## FOREIGN PATENT DOCUMENTS

|    |           |         |
|----|-----------|---------|
| EP | 0629 231  | 12/1994 |
| EP | 0543 356  | 2/1997  |
| EP | 0922 716  | 6/1999  |
| EP | 1391498   | 2/2004  |
| JP | 10-237469 | 9/1998  |
| JP | 10-245574 | 9/1998  |
| JP | 11-181453 | 6/1999  |

|    |             |         |
|----|-------------|---------|
| JP | 2002-338975 | 11/2002 |
| WO | WO 94/00516 | 6/1993  |
| WO | WO 93/14178 | 7/1993  |
| WO | WO 94/17159 | 8/1994  |
| WO | WO 01/38461 | 5/2001  |

## OTHER PUBLICATIONS

English Language Abstract for DE 41 34 347, Apr. 22, 1993.  
 Abstract for DE3443 475, May 28, 1986.  
 Abstract for EP 0203 554, Dec. 3, 1986.  
 Abstract for EP 0254 284, Jan. 27, 1988.  
 Abstract for EP 0271 738, Jun. 22, 1988.  
 Abstract for EP 0543 356, Feb. 12, 1997.  
 Roempp Chemie Lexikon, 9th Ed., (1988-1992) vol. 4, pp. (3351-3354).  
 I. M. El-Gamal, et al., "Polymeric structures as cold flow improvers for waxy residual fuel oil", Fuel 1997, vol. 76, No. 14/15, (1997), Elsevier.  
 Copending U.S. Appl. No. 11/803,786, filed May 16, 2007, to Bettina Siggekow.  
 Copending U.S. Appl. No. 11/803,858, filed May 16, 2007, to Bettina Siggekow.  
 Copending U.S. Appl. No. 11/803,874, filed May 16, 2007, to Bettina Siggekow.  
 Copending U.S. Appl. No. 11/803,798, filed May 16, 2007, to Bettina Siggekow.

**FUEL OILS COMPOSED OF MIDDLE DISTILLATES AND OILS OF VEGETABLE OR ANIMAL ORIGIN AND HAVING IMPROVED COLD FLOW PROPERTIES**

The present invention relates to mineral fuel oils comprising constituents of vegetable or animal origin and having improved cold flow properties, and also to the use of an additive as a cold flow improver for such fuel oils.

In view of decreasing world crude oil reserves and the discussion about the environmentally damaging consequences of the use of fossil and mineral fuels, there is increasing interest in alternative energy sources based on renewable raw materials (biofuels). These include in particular natural oils and fats of vegetable or animal origin. These are generally triglycerides of fatty acids having from 10 to 24 carbon atoms and a calorific value comparable to conventional fuels, but are at the same time regarded as being less harmful to the environment. Biofuels, i.e. fuels derived from animal or vegetable material, are obtained from renewable sources and, when they are combusted, generate only as much CO<sub>2</sub> as had previously been converted to biomass. It has been reported that less carbon dioxide is formed in the course of combustion than by the equivalent amount of crude oil distillate fuel, for example diesel fuel, and that very little sulfur dioxide is formed. In addition, they are biodegradable.

Oils obtained from animal or vegetable, material are mainly metabolism products which include triglycerides of monocarboxylic acids, for example acids having from 10 to 25 carbon atoms, and corresponding to the formula



where R is an aliphatic radical which has from 10 to 25 carbon atoms and may be saturated or unsaturated.

In general, such oils contain glycerides from a series of acids whose number and type vary with the source of the oil, and they may additionally contain phosphoglycerides. Such oils can be obtained by processes known from the prior art.

As a consequence of the sometimes unsatisfactory physical properties of the triglycerides, the industry has applied itself to converting the naturally occurring triglycerides to fatty acid esters of low alcohols such as methanol or ethanol.

A hindrance to the use of fatty acid esters of lower monohydric alcohols as a replacement for diesel fuel alone has been found to be its behavior toward engine parts, especially various sealing materials, which lead time and time again to breakdowns of the engines operated using these fuels produced from renewable raw materials. To circumvent these problems, preference is given to using these oils based on renewable raw materials as an additive to conventional middle distillates.

In addition, when triglycerides and also fatty acid esters of lower monohydric alcohols are used as a replacement for diesel fuel, alone or in a mixture with diesel fuel, a hindrance has been found to be the flow behavior at low temperatures. The causes of this are in particular their content of esters of saturated fatty acids and the high uniformity (less than 10 main components) of these oils in comparison to mineral oil middle distillates. For example, rapeseed oil methyl ester

(RME) has a Cold Filter Plugging Point (CFPP) of -14° C., soya oil methyl ester a CFPP of -5° C. and animal fat a CFPP of +9° C. It has hitherto often been impossible using the prior art additives, on the basis of mineral diesel comprising this ester or these esters, to reliably obtain a CFPP value of -20° C. required for use as a winter diesel in Central Europe, or of -22° C. or lower for special applications. This problem is increased when oils are used which comprise relatively large amounts of the likewise readily available oils of sunflowers and soya.

EP-B-0 665 873 discloses a fuel oil composition which includes a biofuel, a fuel oil based on crude oil and an additive which comprises (a) an oil-soluble ethylene copolymer or (b) a comb polymer or (c) a polar nitrogen compound or (d) a compound in which at least one substantially linear alkyl group having from 10 to 30 carbon atoms is bonded to a nonpolymeric organic radical, in order to provide at least one linear chain of atoms which includes the carbon atoms of the alkyl groups and one or more nonterminal oxygen atoms, or (e) one or more of components (a), (b), (c) and (d).

EP-B-0 629 231 discloses a composition which comprises a relatively large proportion of oil which consists substantially of alkyl esters of fatty acids which are derived from vegetable or animal oils or both, mixed with a small proportion of mineral oil cold flow improvers which comprises one or more of the following:

- (I) comb polymer, the copolymer (which may be esterified) of maleic anhydride or fumaric acid and another ethylenically unsaturated monomer, or polymer or copolymer of  $\alpha$ -olefin, or fumarate or itaconate polymer or copolymer,
- (II) polyoxyalkylene ester, ester/ether or a mixture thereof,
- (III) ethylene/unsaturated ester copolymer,
- (IV) polar, organic, nitrogen-containing paraffin crystal growth inhibitor,
- (V) hydrocarbon polymer,
- (VI) sulfur-carboxyl compounds and
- (VII) aromatic pour point depressant modified with hydrocarbon radicals,

with the proviso that the composition comprises no mixtures of polymeric esters or copolymers of esters of acrylic and/or methacrylic acid which are derived from alcohols having from 1 to 22 carbon atoms.

EP-B-0 543 356 discloses a process for preparing compositions having improved low temperature performance for use as fuels or lubricants, starting from the esters of naturally occurring long-chain fatty acids with monohydric C<sub>1</sub>-C<sub>6</sub>-alcohols (FAE), which comprises

- a) adding PPD additives (pour point depressants) known per se and used for improving the low temperature performance of mineral oils in amounts of from 0.0001 to 10% by weight, based on the long-chain fatty acid esters FAE and
- b) cooling the nonadditized long-chain fatty acid esters FAE to a temperature below the Cold Filter Plugging Point and
- c) removing the resulting precipitates (FAN).

DE-A-40 40 317 discloses mixtures of fatty acid lower alkyl esters having improved cold stability comprising

- a) from 58 to 95% by weight of at least one ester within the iodine number range from 50 to 150 and being derived from fatty acids having from 12 to 22 carbon atoms and lower aliphatic alcohols having from 1 to 4 carbon atoms,
- b) from 4 to 40% by weight of at least one ester of fatty acids having from 6 to 14 carbon atoms and lower aliphatic alcohols having from 1 to 4 carbon atoms and
- c) from 0.1 to 2% by weight of at least one polymeric ester.

EP-B-0 153 176 discloses the use of polymers based on unsaturated dialkyl C<sub>4</sub>-C<sub>8</sub>-dicarboxylates having an average alkyl chain length of from 12 to 14 as cold flow improvers for certain crude oil distillate fuel oils. Mentioned as suitable comonomers are unsaturated esters, in particular vinyl acetate, but also  $\alpha$ -olefins.

EP-B-0 153 177 discloses an additive concentrate which comprises a combination of

I) a copolymer having at least 25% by weight of an n-alkyl ester of a monoethylenically unsaturated C<sub>4</sub>-C<sub>8</sub> mono- or dicarboxylic acid, the average number of carbon atoms in the n-alkyl radicals being 12-14, and another unsaturated ester or an olefin, with

II) another low temperature flow improver for distillate fuel oils.

EP-B-0 746 598 discloses comb polymers as a cold additive in fuel oils which have a cloud point of at most -10° C.

It has hitherto often been impossible using the existing additives to reliably adjust middle distillates comprising fatty acid esters to a CFPP value of -20° C. required for use as a winter diesel in Central Europe or of -22° C. and lower for special applications. An additional problem with the existing additives is lacking sedimentation stability of the additized oils. The paraffins and fatty acid esters precipitating below the cloud point sediment when the oil is stored below the cloud point for a prolonged period and lead to the formation of a phase having poorer cold properties on the bottom of the storage vessel.

It is thus an object of the present invention to provide fuel oils having improved cold properties and comprising middle distillates and fatty acid esters, their CFPP values being at -20° C. and below. Moreover, the sedimentation of precipitated paraffins and fatty acid esters in the course of prolonged storage of the fuel oil should be slowed or prevented in the region of its cloud point or below.

It has now been found that, surprisingly, fuel oils composed of middle distillates and oils of vegetable and/or animal origin, which include an additive comprising ethylene copolymers and certain comb polymers, exhibit excellent cold properties.

The invention thus provides a fuel oil composition F) comprising

F1) a fuel oil of mineral origin and

F2) a fuel oil of vegetable and/or animal origin, and, as a cold additive, the constituents

A) at least one copolymer composed of ethylene and 8-21 mol % of at least one acrylic or vinyl ester having a C<sub>1</sub>-C<sub>18</sub>-alkyl radical and

B) at least one comb polymer containing structural units having C<sub>8</sub>-C<sub>16</sub>-alkyl radicals, the structural units being selected from C<sub>8</sub>-C<sub>16</sub>-alkyl (meth)acrylates, C<sub>8</sub>-C<sub>16</sub>-alkyl vinyl esters, C<sub>8</sub>-C<sub>16</sub>-alkyl vinyl ethers, C<sub>8</sub>-C<sub>16</sub>-alkyl(meth) acrylamides, C<sub>8</sub>-C<sub>16</sub>-alkyl allyl ethers and C<sub>8</sub>-C<sub>16</sub>-diketenes,

where the sum R

$$R = m_1 \cdot \sum_i w_{1i} \cdot n_{1i} + m_2 \cdot \sum_j w_{2j} \cdot n_{2j} + \dots + m_g \cdot \sum_p w_{gp} \cdot n_{gp}$$

of the molar averages of the carbon chain length distributions in the alkyl radicals of the monomers B) is from 11.0 to 14.0,

where

m<sub>1</sub>, m<sub>2</sub>, ..., m<sub>g</sub> are the molar fractions of the abovementioned monomers B) in the polymer, and the sum of the molar fractions m<sub>1</sub> to m<sub>g</sub>=1,

w<sub>1i</sub>, w<sub>1j</sub> ..., w<sub>2i</sub>, w<sub>2j</sub> ..., w<sub>gp</sub> are the proportions by weight of the individual chain lengths i,j, p of the alkyl radicals of the different monomers B) 1 to g, and

n<sub>1i</sub>, n<sub>1j</sub> ..., n<sub>2i</sub>, n<sub>2j</sub> ..., n<sub>gp</sub> are the chain lengths of the alkyl radicals i, j, ..., p of the monomers B) 1 to g.

The invention further provides the use of the above-defined additive comprising constituents A) and B) for improving the cold properties of fuel oil compositions F) comprising fuel oils of mineral (F1) and animal and/or vegetable (F2) origin.

The invention further provides a process for producing fuel oil compositions F) comprising fuel oils of mineral (F1) and animal and/or vegetable (F2) origin, having improved cold flow properties, by adding the above-defined additive comprising constituents A) and B) to the mixture of fuel oils of mineral (F1) and animal and/or vegetable (F2) origin.

Preferred oils of mineral origin are middle distillates. The mixing ratio between the fuel oils of animal and/or vegetable origin (which are also referred to hereinbelow as biofuels) and middle distillates may be between 1:99 and 99:1. Particular preference is given to mixtures which contain from 2 to 50% by volume, in particular from 5 to 40% by volume and especially from 10 to 30% by volume, of biofuels. The inventive additives impart to these mixtures superior cold properties.

In a preferred embodiment of the invention, R assumes values between 11.5 and 13.5, in particular from 12.0 to 13.0.

Suitable ethylene copolymers A) are those which contain from 8 to 21 mol % of one or more vinyl and/or (meth)acrylic esters and from 79 to 92 mol % of ethylene. Particular preference is given to ethylene copolymers having from 10 to 18 mol %, and especially from 12 to 16 mol %, of at least one vinyl ester. Suitable vinyl esters are derived from fatty acids having linear or branched alkyl groups having from 1 to 30 carbon atoms. Examples include vinyl acetate, vinyl propionate, vinyl butyrate, vinyl hexanoate, vinyl heptanoate, vinyl octanoate, vinyl laurate and vinyl stearate, and also esters of vinyl alcohol based on branched fatty acids, such as vinyl isobutyrate, vinyl pivalate, vinyl 2-ethylhexanoate, vinyl isononanoate, vinyl neononanoate, vinyl neodecanoate and vinyl neoundecanoate. Likewise suitable as comonomers are esters of acrylic and methacrylic acids having from 1 to 20 carbon atoms in the alkyl radical, such as methyl (meth) acrylate, ethyl (meth)acrylate, propyl (meth)acrylate, n- and isobutyl (meth)acrylate, and hexyl, octyl, 2-ethylhexyl, decyl, dodecyl, tetradecyl, hexadecyl and octadecyl (meth) acrylate, and also mixtures of two, three, four or else more of these comonomers.

Particularly preferred terpolymers of vinyl 2-ethylhexanoate, of vinyl neononanoate or of vinyl neodecanoate contain, apart from ethylene, preferably from 3.5 to 20 mol %, in particular from 8 to 15 mol %, of vinyl acetate, and from 0.1 to 12 mol %, in particular from 0.2 to 5 mol %, of the particular long-chain vinyl ester, the total comonomer content being between 8 and 21 mol %, preferably between 12 and 18 mol %. In addition to ethylene and from 8 to 18 mol % of vinyl esters, further preferred copolymers additionally contain from 0.5 to 10 mol % of olefins such as propene, butene, isobutylene, hexene, 4-methylpentene, octene, diisobutylene and/or norbornene.

The copolymers A) preferably have molecular weights which correspond to melt viscosities at 140° C. of from 20 to 10 000 mPas, in particular from 30 to 5000 mPas, and especially from 50 to 1000 mPas. The degrees of branching determined by means of <sup>1</sup>H NMR spectroscopy are preferably between 1 and 9 CH<sub>3</sub>/100 CH<sub>2</sub> groups, in particular between

2 and 6 CH<sub>3</sub>/100 CH<sub>2</sub> groups, for example from 2.5 to 5 CH<sub>3</sub>/100 CH<sub>2</sub> groups, which do not stem from the comonomers.

The copolymers (A) can be prepared by customary copolymerization processes, for example suspension polymerization, solution polymerization, gas phase polymerization or high pressure bulk polymerization. Preference is given to carrying out the high pressure bulk polymerization at pressures of from 50 to 400 MPa, preferably from 100 to 300 MPa, and temperatures from 100 to 300° C., preferably from 150 to 220° C. In a particularly preferred preparation variant, the polymerization is effected in a multizone reactor in which the temperature difference between the peroxide feeds along the tubular reactor is kept very low, i.e. <50° C., preferably <30° C., in particular <15° C. The temperature maxima in the individual reaction zones preferably differ by less than 30° C., more preferably by less than 20° C. and especially by less than 10° C.

The reaction of the monomers is initiated by free radical-forming initiators (free radical chain initiators). This substance class includes, for example, oxygen, hydroperoxides, peroxides and azo compounds, such as cumene hydroperoxide, t-butyl hydroperoxide, dilauroyl peroxide, dibenzoyl peroxide, bis(2-ethylhexyl) peroxydicarbonate, t-butyl perpivalate, t-butyl permaleate, t-butyl perbenzoate, dicumyl peroxide, t-butyl cumyl peroxide, di(t-butyl) peroxide, 2,2'-azobis(2-methylpropanonitrile), 2,2'-azobis(2-methylbutyronitrile). The initiators are used individually or as a mixture of two or more substances in amounts of from 0.01 to 20% by weight, preferably from 0.05 to 10% by weight, based on the monomer mixture.

The high pressure bulk polymerization is carried out in known high pressure reactors, for example autoclaves or tubular reactors, batchwise or continuously, and tubular reactors have been found to be particularly useful. Solvents such as aliphatic and/or aromatic hydrocarbons or hydrocarbon mixtures, benzene or toluene may be present in the reaction mixture. Preference is given to the substantially solvent-free procedure. In a preferred embodiment of the polymerization, the mixture of the monomers, the initiator and, if used, the moderator, are fed to a tubular reactor via the reactor entrance and also via one or more side branches. Preferred moderators are, for example, hydrogen, saturated and unsaturated hydrocarbons, for example propane or propene, aldehydes, for example propionaldehyde, n-butyraldehyde or isobutyraldehyde, ketones, for example acetone, methyl ethyl ketone, methyl isobutyl ketone, cyclohexanone, and alcohols, for example butanol. The comonomers and also the moderators may be metered into the reactor either together with ethylene or else separately via sidestreams. The monomer streams may have different compositions (EP-A-0 271 738 and EP-A-0 922 716).

Examples of suitable co- or terpolymers include: ethylene-vinyl acetate copolymers having 10-40% by weight of vinyl acetate and 60-90% by weight of ethylene; the ethylene-vinyl acetate-hexene terpolymers disclosed by DE-A-34 43 475;

the ethylene-vinyl acetate-diisobutylene terpolymers described in EP-B-0 203 554;

the mixture of an ethylene-vinyl acetate-diisobutylene terpolymer and an ethylene/vinyl acetate copolymer disclosed by EP-B-0 254 284;

the mixtures of an ethylene-vinyl acetate copolymer and an ethylene-vinyl acetate-N-vinylpyrrolidone terpolymer disclosed in EP-B-0 405 270;

the ethylene/vinyl acetate/isobutyl vinyl ether terpolymers described in EP-B-0 463 518;

the ethylene/vinyl acetate/vinyl neononanoate or vinyl neodecanoate terpolymers which, apart from ethylene, contain 10-35% by weight of vinyl acetate and 1-25% by weight of the particular neo compound, disclosed by EP-B-0 493 769;

the terpolymers of ethylene, a first vinyl ester having up to 4 carbon atoms and a second vinyl ester which is derived from a branched carboxylic acid having up to 7 carbon atoms or a branched but nontertiary carboxylic acid having from 8 to 15 carbon atoms, described in EP 0778875;

the terpolymers of ethylene, the vinyl ester of one or more aliphatic C<sub>2</sub>-to C<sub>20</sub>-monocarboxylic acids and 4-methylpentene-1, described in DE-A-196 20 118;

the terpolymers of ethylene, the vinyl ester of one or more aliphatic C<sub>2</sub>-to C<sub>20</sub>-monocarboxylic acids and bicyclo [2.2.1]hept-2-ene, disclosed in DE-A-196 20 119;

the terpolymers of ethylene and at least one olefinically unsaturated comonomer which contains one or more hydroxyl groups, described in EP-A-0 926 168.

Preference is given to using mixtures of the same or different ethylene copolymers. The polymers on which the mixtures are based more preferably differ in at least one characteristic. For example, they may contain different comonomers, different comonomer contents, molecular weights and/or degrees of branching. The mixing ratio of the different ethylene copolymers is preferably between 20:1 and 1:20, preferably from 10:1 to 1:10, in particular from 5:1 to 1:5.

The copolymers B are derived from alkyl acrylates, alkyl methacrylates, alkylacrylamides, alkylmethacrylamides, alkyl vinyl esters, alkyl vinyl ethers, alkyl allyl ethers and also alkyl diketenes having from 8 to 16 carbon atoms in the alkyl radical. These comonomers are referred to hereinbelow as comonomers B1).

In a preferred embodiment, the copolymers which make up constituent B are those which contain comonomers which are derived from esters, amides and/or imides of ethylenically unsaturated monocarboxylic acids having from 3 to 8 carbon atoms with alcohols or amines, the alcohols or amines bearing alkyl radicals having from 8 to 16 carbon atoms.

Optionally, the copolymers B) may also contain comonomers B2) which are i) esters, amides and/or imides of ethylenically unsaturated dicarboxylic acids having from 4 to 8 carbon atoms and alcohols or amines having from 8 to 16 carbon atoms in the alkyl radicals, and/or ii) C<sub>10</sub> to C<sub>20</sub> olefins.

The alkyl radicals of the comonomers B1 and B2 are preferably linear, but may also contain minor amounts of branched isomers of up to 30 mol %, preferably up to 20 mol % and in particular from 2 to 5 mol %.

The proportion of the comonomers B1) and optionally B2) in the polymer is preferably more than 50 mol %, in particular more than 70 mol % and especially at least 80 mol %, for example from 90 to 95 mol %.

The proportion of the monomers B2), where present, is preferably less than 80 mol %, in particular less than 50 mol % and especially less than 20 mol %, for example from 2 to 10 mol % of the total amount of the monomers B1) and B2). The polymers B) more preferably consist only of the monomers B1) and optionally B2) which then add up to 100 mol %.

Preferred monomers of the copolymers B) are esters of acrylic acid, methacrylic acid, maleic acid, fumaric acid and itaconic acid with octanol, nonanol, decanol, undecanol, dodecanol, n-tridecanol, isotridecanol, tetradecanol, pentadecanol, hexadecanol and mixtures thereof. Preferred monomers are also amides and optionally imides of these acids with octylamine, nonylamine, decylamine, undecylamine, dode-

cyclamine, tridecylamine, tetradecylamine, pentadecylamine, hexadecylamine and mixtures thereof.

In a preferred embodiment, the copolymers which make up constituent B contain comonomers which are esters and/or ethers of ethylenically unsaturated alcohols having from 2 to 10 carbon atoms, and carboxylic acids or alcohols which bear alkyl radicals having from 8 to 16 carbon atoms.

Such preferred monomers of the copolymers B) are, for example, esters of vinyl alcohol with octanoic acid, 2-ethylhexanoic acid, nonanoic acid, nononanoic acid, decanoic acid, neodecanoic acid, undecanoic acid, neoundecanoic acid, dodecanoic acid, tridecanoic acid, tetradecanoic acid, pentadecanoic acid, hexadecanoic acid and mixtures thereof.

Further preferred monomers of the copolymers B) are, for example, ethers of allyl alcohol and especially of vinyl alcohol with octanol, nonanol, decanol, undecanol, dodecanol, n-tridecanol, isotridecanol, tetradecanol, pentadecanol, hexadecanol and mixtures thereof.

Likewise suitable as comonomers B2 are olefins having 10-20 carbon atoms, preferably having 12-18 carbon atoms and in particular having 10-16 carbon atoms. These are preferably linear  $\alpha$ -olefins having a terminal double bond. In a further preferred embodiment, they are branched olefins, especially oligomers of isobutylene and of propylene having from 10 to 20 carbon atoms.

Side chain length of olefins refers here to the alkyl radical departing from the polymer backbone i.e. the chain length of the monomeric olefin minus the two olefinically bonded carbon atoms. In the case of olefins having nonterminal double bonds, for example olefins having vinylidene moiety, the total chain length of the olefin minus the double bond merging into the polymer backbone correspondingly has to be taken into account.

Further monomers such as alkyl (meth)acrylates, alkyl vinyl esters, alkyl vinyl ethers having from 1 to 5 carbon atoms in the alkyl radical and ethylenically unsaturated free carboxylic acids, for example acrylic acid, methacrylic acid, maleic acid, fumaric acid, itaconic acid and monomers bearing functional groups, for example  $-\text{OH}$ ,  $-\text{SH}$ ,  $-\text{N}-$ ,  $-\text{CN}$ , may likewise be present in the copolymers B in minor amounts of up to 20 mol %, preferably <10 mol %, especially <5 mol %. Also present in minor amounts of up to 20 mol %, preferably <10 mol %, especially <5 mol % may be further comonomers which are copolymerizable with the monomers mentioned, for example allyl polyglycol ethers, styrenes and higher molecular weight olefins such as poly(isobutylene).

Alkyl polyglycol ethers correspond to the general formula



where

$\text{R}^1$  is hydrogen or methyl,

$\text{R}^2$  is hydrogen or  $\text{C}_1\text{-C}_4$ -alkyl,

$m$  is a number from 1 to 100,

$\text{R}^3$  is  $\text{C}_1\text{-C}_{24}$ -alkyl,  $\text{C}_5\text{-C}_{20}$ -cycloalkyl,  $\text{C}_6\text{-C}_{18}$ -aryl or  $-\text{C}(\text{O})-\text{R}^4$ ,

$\text{R}^4$  is  $\text{C}_1\text{-C}_{40}$ -alkyl,  $\text{C}_5\text{-C}_{10}$ -cycloalkyl or  $\text{C}_6\text{-C}_{18}$ -aryl.

All comonomers not falling under the above-specified definitions of B1) and/or B2) are not taken into account in the calculation of the factor R.

The inventive polymers may be prepared by direct polymerization from the monomers mentioned in known polymerization processes such as bulk, solution, emulsion, suspension or precipitation polymerization.

- 5 Equally, they may be prepared by derivatizing a base polymer bearing, for example, acid or hydroxyl groups with appropriate fatty acids, fatty alcohols or fatty amines having from 8 to 16 carbon atoms in the alkyl radical. The esterifications, etherifications, amidations and/or imidations are  
 10 effected by known condensation processes. The derivatization may be complete or partial. Partially esterified or amidized, acid-based polymers have (without solvent) acid numbers of preferably 60-140 mg KOH/g and especially of 80-120 mg KOH/g. Copolymers having acid numbers of less  
 15 than 80 mg KOH/g, especially less than 60 mg KOH/g are regarded as being fully derivatized. Polymers bearing partially esterified or etherified hydroxyl groups have OH numbers of from 40 to 200 mg KOH/g, preferably from 60 to 150 mg KOH/g; copolymers having hydroxyl numbers of less  
 20 than 60 mg KOH/g and in particular less than 40 mg KOH/g are regarded as being fully derivatized. Particular preference is given to partially derivatized polymers.

Polymers which bear acid groups and are suitable for derivatization with fatty alcohols and/or amines to give esters  
 25 and/or amides are homo- and copolymers of ethylenically unsaturated carboxylic acids, for example acrylic acid, methacrylic acid, maleic acid, fumaric acid, itaconic acid or reactive equivalents thereof, such as lower esters or anhydrides, for example methyl methacrylates and maleic anhydride,  
 30 with one another and also with further monomers copolymerizable with these acids. Suitable examples are poly(acrylic acid), poly(methacrylic acid), poly(maleic acid), poly(maleic anhydride), poly(acrylic acid-co-maleic acid).

Suitable fatty alcohols and fatty amines are in particular  
 35 linear, but they may also contain minor amounts, for example up to 30% by weight, preferably up to 20% by weight and especially up to 10% by weight, of branched alkyl radicals. The branches are preferably in the 1- or 2-position. Either shorter- or longer-chain fatty alcohols or fatty amines may be  
 40 used, but their proportion is preferably below 20 mol % and especially below 10 mol %, for example between 1 and 5 mol %, based on the total amount of the amines used.

Particularly preferred fatty alcohols are octanol, decanol, undecanol, dodecanol, tridecanol, tetradecanol, pentadecanol and hexadecanol.

Suitable amines are primary and secondary amines having  
 45 one or two  $\text{C}_8\text{-C}_{16}$ -alkyl radicals. They may bear one, two or three amino groups which are bonded via alkylene radicals having two or three carbon atoms. Preference is given to monoamines. Particularly preferred primary amines are octylamine, 2-ethylhexylamine, decylamine, undecylamine, dodecylamine, n-tridecylamine, isotridecylamine, tetradecylamine, pentadecylamine, hexadecylamine and mixtures thereof. Preferred secondary amines are dioctylamine,  
 50 dinonylamine, didecylamine, didodecylamine, ditetradecylamine, dihexadecylamine, and also amines having different alkyl chain lengths, for example N-octyl-N-decylamine, N-decyl-N-dodecylamine, N-decyl-N-tetradecylamine, N-decyl-N-hexadecylamine, N-dodecyl-N-tetradecylamine,  
 55 N-dodecyl-N-hexadecylamine, N-tetradecyl-N-hexadecylamine. Also suitable in accordance with the invention are secondary amines which, in addition to a  $\text{C}_8\text{-C}_{16}$ -alkyl radical, bear shorter side chains having from 1 to 5 carbon atoms, for example methyl or ethyl groups. In the case of secondary amines, it is the average of the alkyl chain lengths of from  $\text{C}_8$  to  $\text{C}_{16}$  that is taken into account as the alkyl chain length n for the calculation of the Q factor.

Neither shorter nor longer alkyl radicals, where present, are taken into account in the calculation, since they do not contribute to the effectiveness of the additives. The proportion of shorter and longer alkyl chains is therefore preferably below 20 mol %, preferably below 10 mol %, based on the total amount of amine used. Particular preference is given to amides and imides derived from primary monoamines.

Polymers which bear hydroxyl groups and are particularly suitable for the derivatization with fatty acids and/or fatty alcohols to give esters and/or ethers are homo- and copolymers of monomers bearing hydroxyl groups such as vinyl alcohol, allyl alcohol or else hydroxyethyl acrylate, hydroxyethyl methacrylate, hydroxypropyl acrylate and hydroxypropyl methacrylate. Suitable fatty acids have from 8 to 16 carbon atoms in the alkyl radical. The alkyl radical is substantially linear, but may also contain minor amounts, for example up to 30% by weight, preferably up to 20% by weight and especially up to 10% by weight, of branched isomers. Particularly suitable are nonanoic acid, decanoic acid, undecanoic acid, dodecanoic acid, tridecanoic acid, tetradecanoic acid, pentadecanoic acid, hexadecanoic acid, heptadecanoic acid and octadecanoic acid and nonadecanoic acid and mixtures thereof.

The use of mixtures of different fatty acids, alcohols and/or amines in the esterification, etherification, amidation or imidation allows the effectiveness of the inventive additives to be further adapted to specific fatty acid ester compositions.

The molecular weights of the inventive copolymers B are between 1000 and 100 000 g/mol, in particular between 2000 and 50 000 g/mol and in particular between 2500 and 25 000 g/mol, measured by means of gel-permeation chromatography (GPC) against poly(styrene). Inventive copolymers B have to be oil-soluble in dosages relevant to the practice, i.e. they have to dissolve without residue in the oil to be additized at 50° C.

In a preferred embodiment, mixtures of the copolymers B according to the invention are used, with the proviso that the average of the R values of the mixing components in turn assumes values of from 11.0 to 14.0, preferably from 11.5 to 13.5 and in particular values from 12.0 to 13.0.

The mixing ratio of the additives A and B according to the invention is (in parts by weight) from 20:1 to 1:20, preferably from 10:1 to 1:10, in particular from 5:1 to 1:2.

The additives according to the invention are added to oils in amounts of from 0.001 to 5% by weight, preferably from 0.005 to 1% by weight and especially from 0.01 to 0.5% by weight. They may be used as such or else dissolved or dispersed in solvents, for example aliphatic and/or aromatic hydrocarbons or hydrocarbon mixtures, for example toluene, xylene, ethylbenzene, decane, pentadecane, petroleum fractions, kerosene, naphtha, diesel, heating oil, isoparaffins or commercial solvent mixtures such as Solvent Naphtha, ®Shellsol AB, ®Solvesso 150, ®Solvesso 200, ®Exxsol, ®Isopar and ®Shellsol D types. They are preferably dissolved in fuel oil of animal or vegetable origin based on fatty acid alkyl esters. The additives according to the invention preferably comprise 1-80%, especially 10-70%, in particular 25-60%, of solvent.

In a preferred embodiment, the fuel oil F2, which is frequently also referred to as biodiesel or biofuel, is a fatty acid alkyl ester composed of fatty acids having from 12 to 24 carbon atoms and alcohols having from 1 to 4 carbon atoms. Typically, a relatively large portion of the fatty acids contains one, two or three double bonds.

Examples of oils F2 which are derived from animal or vegetable material and can be used in accordance with the invention are rapeseed oil, coriander oil, soya oil, cottonseed

oil, sunflower oil, castor oil, olive oil, peanut oil, maize oil, almond oil, palmseed oil, coconut oil, mustardseed oil, bovine tallow, bone oil, fish oils and used cooking oils. Further examples include oils which are derived from wheat, jute, sesame, shea tree nut, arachis oil and linseed oil. The fatty acid alkyl esters also referred to as biodiesel can be derived from these oils by processes disclosed by the prior art. Preference is given to rapeseed oil, which is a mixture of fatty acids partially esterified with glycerol, since it is obtainable in large amounts and is obtainable in a simple manner by extractive pressing of rapeseeds. In addition, preference is given to the likewise widely available oils of sunflowers and soya, and also to their mixtures with rapeseed oil.

Particularly suitable biofuels F2) are lower alkyl esters of fatty acids. These include, for example, commercially available mixtures of the ethyl, propyl, butyl and in particular methyl esters of fatty acids having from 14 to 22 carbon atoms, for example of lauric acid, myristic acid, Dalmatic acid, palmitolic acid, stearic acid, oleic acid, elaidic acid, petroselic acid, ricinolic acid, elaeostearic acid, linolic acid, linolenic acid, eicosanoic acid, gadoleic acid, docosanoic acid or erucic acid, each of which preferably has an iodine number of from 50 to 150, in particular from 90 to 125. Mixtures having particularly advantageous properties are those which comprise mainly, i.e. comprise at least 50% by weight, of methyl esters of fatty acids having from 16 to 22 carbon atoms, and 1, 2 or 3 double bonds. The preferred lower alkyl esters of fatty acids are the methyl esters of oleic acid, linoleic acid, linolenic acid and erucic acid.

Commercial mixtures of the type mentioned are obtained, for example, by hydrolyzing and esterifying, or by transesterifying, animal and vegetable fats and oils with lower aliphatic alcohols. Equally suitable as starting materials are used cooking oils. To prepare lower alkyl esters of fatty acids, it is advantageous to start from fats and oils having a high iodine number, for example sunflower oil, rapeseed oil, coriander oil, castor oil, soya oil, cottonseed oil, peanut oil or bovine tallow. Preference is given to lower alkyl esters of fatty acids based on a novel type of rapeseed oil, more than 80% by weight of whose fatty acid component is derived from unsaturated fatty acids having 18 carbon atoms.

A biofuel is therefore an oil which is obtained from vegetable or animal material or both or a derivative thereof which can be used as a fuel and in particular as a diesel or heating oil. Although many of the above oils can be used as biofuels, preference is given to vegetable oil derivatives, and particularly preferred biofuels are alkyl ester derivatives of rapeseed oil, cottonseed oil, soya oil, sunflower oil, olive oil or palm oil, and very particular preference is given to rapeseed oil methyl ester, sunflower oil methyl ester and soya oil methyl ester. Particularly preferred as a biofuel or as a component in biofuel are additionally also used fatty esters, for example used fatty acid methyl ester.

Suitable mineral oil components F1 are in particular middle distillates which are obtained by distilling crude oil and boil in the range from 120 to 450° C., for example kerosene, jet fuel, diesel and heating oil. Preference is given to using those middle distillates which contain 0.05% by weight of sulfur and less, more preferably less than 350 ppm of sulfur, in particular less than 200 ppm of sulfur and in special cases less than 50 ppm of sulfur, for example less than 10 ppm of sulfur. These are generally those middle distillates which have been subjected to refining under hydrogenating conditions, and therefore contain only small proportions of polycyclic and polar compounds. They are preferably those middle distillates which have 95% distillation points below 370° C., in particular 350° C. and in special cases below 330°

## 11

C. Synthetic fuels, as obtainable, for example, by the Fischer-Tropsch process, are also suitable as middle distillates.

The additive can be added to the oil to be additized in accordance with prior art processes. When more than one additive component or coadditive component is to be used, such components can be introduced into the oil together or separately in any desired combination and sequence.

The inventive additives allow the CFPP value of mixtures of biodiesel and mineral oils to be improved much more efficiently than using the known prior art additives. The inventive additives are particularly advantageous in oil mixtures whose mineral oil component F1) has a boiling range between the 20% and the 90% distillation point of less than 120° C., in particular of less than 110° C. and especially of less than 100° C. In addition, they are particularly advantageous in oil mixtures whose mineral oil component F1) has a cloud point of below -4° C., in particular from -6° C. to -20° C., for example from -7° C. to -9° C., as required for use in winter in particular. Equally, the pour point of the inventive mixtures is reduced by the addition of the inventive additives. The inventive additives are particularly advantageous in oil mixtures which contain more than 2% by volume of biofuel F2, preferably more than 5% by volume of biofuel F2 and especially more than 10% by volume of biofuel F2, for example from 15 to 35% by volume of biofuel F2. The inventive additives are additionally particularly advantageous in problematic oils whose biofuel component F2 contains a high proportion of esters of saturated fatty acids of more than 4%, in particular of more than 5% and especially having from 7 to 25%, for example having from 8 to 20%, as present, for example, in oils from sunflowers and soya. Such biofuels preferably have a cloud point of above -5° C. and especially above -3° C. Oil mixtures F) in which the inventive additives exhibit particularly advantageous action preferably have cloud points of above -9° C. and especially of above -6° C. It is thus also possible using the inventive additives to adjust oil mixtures comprising rapeseed oil methyl ester and sunflower and/or soya oil fatty acid methyl ester to CFPP values of -22° C. and below.

To prepare additive packages for specific solutions to problems, the inventive additives can also be used together with one or more oil-soluble coadditives which alone improve the cold flow properties of crude oils, lubricant oils or fuel oils. Examples of such coadditives are polar compounds which differ from the inventive polymers B and bring about paraffin dispersion (paraffin dispersants), alkylphenol condensates, esters and ethers of polyoxyalkylene compounds, olefin copolymers, and also oil-soluble amphiphiles.

For instance, the inventive additives may be used in a mixture with paraffin dispersants to further reduce the sedimentation under cold conditions of precipitated paraffins and fatty acid esters. Paraffin dispersants reduce the size of the paraffin and fatty acid ester crystals and have the effect that the paraffin particles do not separate but remain dispersed colloidally with a distinctly reduced tendency to sedimentation. Useful paraffin dispersants have been found to be both low molecular weight and polymeric oil-soluble compounds having ionic or polar groups, for example amine salts and/or amides. Particularly preferred paraffin dispersants comprise reaction products of fatty amines having alkyl radicals having from 18 to 24 carbon atoms, in particular with secondary fatty amines such as ditallow fat amine, distearylamine and dibehenylamine with carboxylic acids and derivatives thereof. Particularly useful paraffin dispersants have been found to be those obtained by reacting aliphatic or aromatic amines, preferably long-chain aliphatic amines, with aliphatic or aromatic mono-, di-, tri- or tetracarboxylic acids or their anhydrides

## 12

(cf. U.S. Pat. No. 4,211,534). Equally suitable paraffin dispersants are amides and ammonium salts of aminoalkylene-polycarboxylic acids such as nitrilotriacetic acid or ethylenediaminetetraacetic acid with secondary amines (cf. EP 0 398 101). Other paraffin dispersants are copolymers of maleic anhydride and  $\alpha,\beta$ -unsaturated compounds which may optionally be reacted with primary monoalkylamines and/or aliphatic alcohols (cf. EP 0 154 177) and the reaction products of alkenyl-spiro-bis lactones with amines (cf. EP 0 413 279 B1) and, according to EP 0 606 055 A2, reaction products of terpolymers based on  $\alpha,\beta$ -unsaturated dicarboxylic anhydrides,  $\alpha,\beta$ -unsaturated compounds and polyoxyalkylene ethers of lower unsaturated alcohols.

Alkylphenol-aldehyde resins are described, for example, in Römpf Chemie Lexikon, 9th edition, Thieme Verlag 1988-92, volume 4, p. 3351 ff. In the alkylphenol-aldehyde resins which can be used in the inventive adjuvants, the alkyl radicals of the o- or p-alkylphenol may be the same or different and have 1-50, preferably 1-20, in particular 4-12, carbon atoms; they are preferably n-, iso- and tert-butyl, n- and isopentyl, n- and isohexyl, n- and isoctyl, n- and isononyl, n- and isodecyl, n- and isododecyl and octadecyl. The aliphatic aldehyde in the alkylphenol-aldehyde resin preferably has 1-4 carbon atoms. Particularly preferred aldehydes are formaldehyde, acetaldehyde and butyraldehyde, in particular formaldehyde. The molecular weight of the alkylphenol-aldehyde resins is 400-10 000 g/mol, preferably 400-5000 g/mol. A prerequisite is that the resins are oil-soluble.

In a preferred embodiment of the invention, these alkylphenol-formaldehyde resins are those which contain oligo- or polymers having a repeating structural unit of the formula



where R<sup>5</sup> is C<sub>1</sub>-C<sub>50</sub>-alkyl or -alkenyl and n is a number from 2 to 100. R<sup>5</sup> is preferably C<sub>4</sub>-C<sub>20</sub>-alkyl or -alkenyl and in particular C<sub>6</sub>-C<sub>16</sub>-alkyl or -alkenyl. n is preferably a number from 4 to 50 and especially a number from 5 to 25.

Further suitable flow improvers are polyoxyalkylene compounds, for example esters, ethers and ether/esters which bear at least one alkyl radical having from 12 to 30 carbon atoms. When the alkyl groups stem radicals come from a fatty alcohol, the rest of the compound stems from a polyacid.

Suitable polyols are polyethylene glycols, polypropylene glycols, polybutylene glycols and their copolymers having a molecular weight of from approx. 100 to approx. 5000, preferably from 200 to 2000. Also suitable are alkoxylates of polyols, for example glycerol, trimethylolpropane, pentaerythritol, neopentyl glycol, and also the oligomers obtainable therefrom by condensation and having from 2 to 10 monomer units, for example polyglycerol. Preferred alkoxylates are those having from 1 to 100 mol, in particular from 5 to 50 mol, of ethylene oxide, propylene oxide and/or butylene oxide per mole of polyol. Particular preference is given to esters.

Fatty acids having from 12 to 26 carbon atoms are preferably used for reaction with the polyols to form the ester additives, although preference is given to using C<sub>18</sub> to C<sub>24</sub> fatty acids, especially stearic acid and behenic acid. The esters can also be prepared by esterification of polyoxyalkylated alcohols. Preference is given to fully esterified polyoxyalkylated polyols having molecular weights of from 150 to

2000, preferably from 200 to 1500. PEG-600 dibehenate and glycerol-ethylene glycol tribehenate are particularly suitable.

Olefin polymers suitable as a constituent of the inventive additive may be derived directly from monoethylenically unsaturated monomers or be prepared indirectly by hydrogenating polymers which are derived from polyunsaturated monomers such as isoprene or butadiene. In addition to ethylene, preferred copolymers contain structural units which are derived from  $\alpha$ -olefins having from 3 to 24 carbon atoms and molecular weights of up to 120 000. Preferred  $\alpha$ -olefins are propylene, butene, isobutene, n-hexene, isohexene, noctene, isoctene, n-decene, isodecene. The comonomer content of olefins is preferably between 15 and 50 mol %, more preferably between 20 and 35 mol % and especially between 30 and 45 mol %. These copolymers may also contain small amounts, for example up to 10 mol %, of further comonomers, for example nonterminal olefins or nonconjugated olefins. Preference is given to ethylene-propylene copolymers. The olefin copolymers may be prepared by known methods, for example by means of Ziegler or metallocene catalysts.

Further suitable olefin copolymers are block copolymers which contain blocks of olefinically unsaturated aromatic monomers A and blocks of hydrogenated polyolefins B. Particularly suitable block copolymers have the structure (AB)<sub>n</sub> A and (AB)<sub>m</sub>, where n is a number between 1 and 10 and m is a number between 2 and 10.

The mixing ratio (in parts by weight) of the inventive additives with paraffin dispersants, comb polymers, alkylphenol condensates, polyoxalkylene derivatives and olefin copolymers respectively is in each case from 1:10 to 20:1, preferably from 1:1 to 10:1, for example from 1:1 to 4:1.

The additives may be used alone or else together with other additives, for example with other pour point depressants or dewaxing assistants, with antioxidants, cetane number improvers, dehazers, deemulsifiers, detergents, dispersants, antifoams, dyes, corrosion inhibitors, conductivity improvers, sludge inhibitors, odorants and/or additives for lowering the cloud point.

#### EXAMPLES

##### Characterization of the Test Oils:

The CFPP value is determined to EN 116 and the cloud point to ISO 3015. Both properties are determined in ° C.

TABLE 1

| Characterization of the biofuels used (F2) |                                                           |      |         |  |
|--------------------------------------------|-----------------------------------------------------------|------|---------|--|
| Oil No.                                    |                                                           | CP   | CFPP    |  |
| E 1                                        | Rapeseed oil methyl ester                                 | -2.3 | -14° C. |  |
| E 2                                        | 90% rapeseed oil methyl ester + 10% soya oil methyl ester | -2.0 | -8° C.  |  |

TABLE 2

Carbon chain distribution of the fatty acid methyl esters used to prepare the test oils (main constituents; area % by GC):

|      | C <sub>16</sub> | C <sub>16'</sub> | C <sub>18</sub> | C <sub>18'</sub> | C <sub>18''</sub> | C <sub>18'''</sub> | C <sub>20</sub> | C <sub>20'</sub> | C <sub>22</sub> | $\Sigma$ | saturated |
|------|-----------------|------------------|-----------------|------------------|-------------------|--------------------|-----------------|------------------|-----------------|----------|-----------|
| RME  | 4.5             | 0.5              | 1.7             | 61.6             | 18.4              | 8.7                | 0.7             | 1.5              | 0.4             | 7.3      |           |
| Soya | 10.4            | 0.1              | 4.1             | 24.8             | 51.3              | 6.9                | 0.5             | 0.4              | 0.4             | 15.4     |           |
| ME   |                 |                  |                 |                  |                   |                    |                 |                  |                 |          |           |

RME = Rapeseed oil methyl ester;  
SoyaME = Soya oil methyl ester

TABLE 3

| 5  | Characterization of the mineral oils used (F1) |          |          |
|----|------------------------------------------------|----------|----------|
|    | D1                                             | D2       |          |
| 10 | Initial boiling point                          | 193° C.  | 181° C.  |
|    | 20% distillation                               | 230° C.  | 235° C.  |
|    | 90% distillation                               | 332° C.  | 344° C.  |
|    | 95% distillation                               | 348° C.  | 361° C.  |
| 15 | (90-20)% distillation                          | 102° C.  | 109° C.  |
|    | Cloud point                                    | -6.0° C. | -8.2° C. |
|    | CFPP                                           | -8° C.   | -12° C.  |
| 20 | Sulfur content                                 | 20 ppm   | 32 ppm   |

The following additives were used:

##### Ethylene copolymers A

The ethylene copolymers used are commercial products having the characteristics specified in Table 4. The products were used as 65% dilutions in kerosene.

TABLE 4

| Characterization of the ethylene copolymers used (A) |                                                                                                                                 |          |                                      |
|------------------------------------------------------|---------------------------------------------------------------------------------------------------------------------------------|----------|--------------------------------------|
| Example                                              | Comonomer(s)                                                                                                                    | V140     | CH <sub>3</sub> /100 CH <sub>2</sub> |
| 35 A1                                                | 13.6 mol % of vinyl acetate                                                                                                     | 130 mPas | 3.7                                  |
| A2                                                   | 13.7 mol % of vinyl acetate and 1.4 mol % of vinyl neodecanoate                                                                 | 105 mPas | 5.3                                  |
| 40 A3                                                | i) 14.0 mol % of vinyl acetate and 1.6 mol % of vinyl neodecanoate and ii) 12.9 mol % of vinyl acetate in a i):ii) ratio of 6:1 | 97 mPas  | 4.7                                  |
|                                                      |                                                                                                                                 | 145 mPas | 5.4                                  |

##### Comb polymers B

Different co- and terpolymers having the molar ratios, specified in Table 3, of the monomers and the factors R calculated therefrom were investigated. The polymers were used as 50% dilutions in a higher-boiling aromatic solvent. The acid numbers determined relate to at these 50% dilutions.

TABLE 5

Characterization of the comb polymers used (B)

| Example     | Comonomers                                                                                                                                     | R    | Acid number [mg KOH/g] |
|-------------|------------------------------------------------------------------------------------------------------------------------------------------------|------|------------------------|
| B1          | Poly(dodecyl acrylate-co-tetradecyl acrylate) composed of 70% dodecyl acrylate and 30% tetradecyl acrylate and having Mw 10 500                | 12.6 | 1.2                    |
| B2          | Poly(dodecyl methacrylate) having Mw 22 000                                                                                                    | 12.0 | 1.7                    |
| B3          | Poly(2-ethylhexanoate-co-tetradecyl acrylate) composed of 10% 2-ethylhexyl acrylate and 90% tetradecyl acrylate and having Mw 6400             | 13.4 | 10                     |
| B4          | Poly(dodecyl vinyl ether-co-decyl methacrylate) composed of equal proportions of dodecyl vinyl ether and decyl methacrylate and having Mw 5200 | 11.0 | 2.8                    |
| B5          | Poly(acrylic acid) esterified with mixture composed of 75% dodecanol and 25% hexadecanol, Mw 15 000                                            | 13.0 | 43                     |
| B6          | Poly(acrylic acid) esterified with mixture of 40% decanol, 30% dodecanol and 30% tetradecanol, Mw 24 000                                       | 11.8 | 51                     |
| B7          | Poly(acrylic acid-co-maleic acid) esterified with mixture of 55% decanol and 45% hexadecanol, Mw 19 000                                        | 12.7 | 34                     |
| B8 (comp.)  | Poly(decyl acrylate) having Mw 19 000                                                                                                          | 10.0 | 2.3                    |
| B9 (comp.)  | Poly(tetradecyl acrylate-co-hexadecyl acrylate) having equal proportions of tetradecyl and hexadecyl acrylate, Mw 24 000                       | 15.0 | 1.6                    |
| B10 (comp.) | Alternating poly(ditetradecyl fumarate-alt-vinyl acetate)                                                                                      | n.a. | 0.4                    |

n.a. = not applicable

(comp.) = comparative example

## Further flow improvers

The further flow improvers used C are commercial products having the characteristics specified in Table 6. The products were used as 50% dilutions in Solvent Naphtha.

TABLE 6

| Characterization of the further flow improvers used |                                                                                                                                                                                     |    |
|-----------------------------------------------------|-------------------------------------------------------------------------------------------------------------------------------------------------------------------------------------|----|
| C3                                                  | Reaction product of a copolymer composed of C <sub>14</sub> /C <sub>16</sub> olefin and maleic anhydride with 2 equivalents of secondary tallow fat amine per maleic anhydride unit | 35 |
| C4                                                  | Reaction product of phthalic anhydride with 2 equivalents of di(hydrogenated tallow fat amine) to give an amide ammonium salt                                                       | 45 |
| C5                                                  | Nonylphenol resin prepared by condensation of a mixture of dodecylphenol with formaldehyde, Mw 2000 g/mol                                                                           | 50 |
| C6                                                  | Mixture of 2 parts of C3 and 1 part of C5                                                                                                                                           |    |
| C7                                                  | Mixture of equal parts of C4 and C5                                                                                                                                                 |    |

## Effectiveness of the additives

The CFPP value (to EN 116, in °C.) of different biofuels as per the above table was determined after addition of 1200 ppm, 1500 ppm and 2000 ppm of additive mixture. Percentages are based on parts by weight in the particular mixtures. The results reproduced in Tables 5 to 7 show that the comb polymers having the inventive factor Q achieve outstanding CFPP reductions even at low dosages and offer additional potential at higher dosages.

TABLE 7

| CFPP testing in a mixture of 75% by volume of test oil D1 and 25% by volume of test oil E1 (CP = -5.2° C.; CFPP = -9° C.) |               |                        |      |                                      |         |         |         |
|---------------------------------------------------------------------------------------------------------------------------|---------------|------------------------|------|--------------------------------------|---------|---------|---------|
| Ex.                                                                                                                       | Flow improver | polymer/coadditive     | Comb | CFPP after addition of flow improver |         |         |         |
|                                                                                                                           |               |                        |      | 50 ppm                               | 100 ppm | 150 ppm | 200 ppm |
| 1                                                                                                                         | A2            | 150 ppm B4             | -13  | -18                                  | -19     | -20     |         |
| 2                                                                                                                         | A1            | 100 ppm B6             | -17  | -20                                  | -19     | -21     |         |
| 3                                                                                                                         | A2            | 150 ppm B2             | -18  | -20                                  | -22     | -22     |         |
| 4                                                                                                                         | A2            | 150 ppm B1             | -19  | -21                                  | -21     | -23     |         |
| 5                                                                                                                         | A1            | 100 ppm B7             | -20  | -20                                  | -22     | -23     |         |
| 6                                                                                                                         | A1            | 150 ppm B5             | -19  | -21                                  | -20     | -22     |         |
| 7                                                                                                                         | A2            | 150 ppm B3             | -16  | -18                                  | -19     | -21     |         |
| 8                                                                                                                         | A2            | 75 ppm B7<br>75 ppm A4 | -19  | -22                                  | -23     | -25     |         |
| 9 (comp.)                                                                                                                 | A2            | 150 ppm B8             | -11  | -14                                  | -16     | -17     |         |
| 10 (comp.)                                                                                                                | A2            | 150 ppm B9             | -9   | -10                                  | -13     | -16     |         |
| 11 (comp.)                                                                                                                | A2            | 150 ppm B10            | -10  | -11                                  | -15     | -20     |         |
| 13 (comp.)                                                                                                                | A2            | —                      | -11  | -16                                  | -17     | -19     |         |

55

TABLE 8

| CFPP testing in a mixture of 70% by volume of test oil D2 and 30% by volume of test oil E2 (CP = -5.8° C.; CFPP = -12° C.) |                    |              |            |         |         |         |     |
|----------------------------------------------------------------------------------------------------------------------------|--------------------|--------------|------------|---------|---------|---------|-----|
| Ex.                                                                                                                        | Ethylene copolymer | Comb polymer | Coadditive | CFPP    |         |         |     |
|                                                                                                                            |                    |              |            | 100 ppm | 150 ppm | 200 ppm |     |
| 14                                                                                                                         | 80% A3             | 20% B4       | 150 ppm C6 | -18     | -20     | -22     | -24 |
| 15                                                                                                                         | 80% A3             | 20% B6       | 150 ppm C6 | -20     | -21     | -24     | -25 |
| 16                                                                                                                         | 80% A3             | 20% B2       | 150 ppm C6 | -20     | -21     | -23     | -26 |
| 17                                                                                                                         | 80% A3             | 20% B1       | 150 ppm C6 | -21     | -22     | -25     | -27 |

TABLE 8-continued

| Ex.     | Ethylene copolymer | Comb polymer | Coadditive | CFPP    |         |         |         |
|---------|--------------------|--------------|------------|---------|---------|---------|---------|
|         |                    |              |            | 100 ppm | 150 ppm | 200 ppm | 300 ppm |
| 18      | 75% A3             | 25% B7       | 150 ppm C6 | -20     | -20     | -23     | -26     |
| 19      | 85% A1             | 15% B5       | 150 ppm C6 | -20     | -22     | -24     | -27     |
| 20      | 80% A1             | 20% B3       | 150 ppm C7 | -19     | -21     | -23     | -25     |
| 21      | 80% A3             | 20% B8       | 150 ppm C6 | -17     | -18     | -19     | -21     |
| (comp.) |                    |              |            |         |         |         |         |
| 22      | 80% A1             | 20% B9       | 150 ppm C6 | -11     | -16     | -19     | -19     |
| (comp.) |                    |              |            |         |         |         |         |
| 23      | 80% A1             | 20% B10      | 150 ppm C7 | -15     | -16     | -18     | -22     |
| (comp.) |                    |              |            |         |         |         |         |
| 24      | 100% A1            | —            | 150 ppm C6 | -18     | -19     | -20     | -22     |
| (comp.) |                    |              |            |         |         |         |         |

In this test series, in each case a constant amount of coaditive and the specified amount of a mixture of ethylene copolymer and comb polymer were added to the oil.

What is claimed is:

1. A fuel oil composition F) comprising
  - F1) a fuel oil of mineral origin and
  - F2) a fuel oil of vegetable and/or animal origin, and, as a cold additive, the constituents
- A) at least one copolymer composed of ethylene and 8-21 mol % of at least one comonomer of acrylic or vinyl ester having a C<sub>1</sub>-C<sub>18</sub>-alkyl radical and
- B) at least one comb polymer containing structural units of monomers having C<sub>8</sub>-C<sub>16</sub>-alkyl radicals, the monomers being selected from the group consisting of C<sub>8</sub>-C<sub>16</sub>-alkyl(meth)acrylates, C<sub>8</sub>-C<sub>16</sub>-alkyl vinyl esters, C<sub>8</sub>-C<sub>16</sub>-alkyl vinyl ethers, C<sub>8</sub>-C<sub>16</sub>-alkyl(meth)acrylamides, C<sub>8</sub>-C<sub>16</sub>-alkyl allyl ethers, C<sub>8</sub>-C<sub>16</sub>-diketenes, and mixtures thereof,

where the sum R

$$R = m_1 \cdot \sum_i w_{1i} \cdot n_{1i} + m_2 \cdot \sum_j w_{2j} \cdot n_{2j} + \dots + m_g \cdot \sum_p w_{gp} \cdot n_{gp}$$

of molar averages of carbon chain length distributions in the C<sub>8</sub>-C<sub>16</sub>-alkyl radicals of the monomers of comb polymer B) is from 11.0 to 14.0,

where

m<sub>1</sub>, m<sub>2</sub>, . . . m<sub>g</sub> are molar fractions of the monomers of comb polymer B) in the polymer, and the sum of the molar fractions m<sub>1</sub> to m<sub>g</sub>=1,

W<sub>1i</sub>, W<sub>1j</sub>, W<sub>2i</sub>, W<sub>2j</sub> . . . W<sub>gp</sub> are the proportions by weight of individual carbon chain lengths i, j, p of the C<sub>8</sub>-C<sub>16</sub>-alkyl radicals of the different monomers of comb polymer B) 1 to g, and

n<sub>1i</sub>, n<sub>1j</sub>, n<sub>2i</sub>, n<sub>2j</sub> . . . n<sub>gp</sub> are the chain lengths of the C<sub>8</sub>-C<sub>16</sub>-alkyl radicals i, j, . . . p of the monomers of comb polymer B) 1 to g.

2. A fuel oil composition as claimed in claim 1, wherein R is from 11.5 to 13.5.

3. A fuel oil composition of claim 1, wherein constituent A, apart from ethylene, contains from 3.5 to 20 mol % of a first comonomer consisting of vinyl acetate and from 0.1 to 12 mol % of a second comonomer selected from the group consisting of vinyl neononanoate, vinyl neodecanoate, vinyl 2-ethylhex-

## 18

anoate, and mixtures thereof, and a total comonomer content of constituent A is between 8 and 21 mol %.

4. A fuel oil composition of claim 1, wherein constituent A comprises a copolymer of ethylene and from 8 to 18 mol % of vinyl esters, and from 0.5 to 10 mol % of olefins selected from the group consisting of propene, butene, isobutylene, hexene, 4-methylpentene, octene, diisobutylene, norbornene, and mixtures thereof.

5. A fuel oil composition of claim 1, wherein constituent A has a melt viscosity between 20 and 10 000 mPas.

6. A fuel oil composition of claim 1, wherein constituent A has a degree of branching between 1 and 9 CH<sub>3</sub>/100 CH<sub>2</sub> groups which do not stem from the comonomers.

7. A fuel oil composition of claim 1, wherein the copolymers which make up constituent B comprise comonomers which are derived from esters or amides of ethylenically unsaturated monocarboxylic acids having from 3 to 8 carbon atoms with alcohols or amines, the alcohols or amines bearing alkyl radicals having from 8 to 16 carbon atoms.

8. A fuel oil composition of claim 1, wherein copolymers B) contain up to 50 mol % of comonomers B2) which comprise

i) selected from the group consisting of esters, amides, imides and mixtures thereof of ethylenically unsaturated dicarboxylic acids having from 4 to 8 carbon atoms and alcohols or amines having from 8 to 16 carbon atoms in the alkyl radicals or,

ii) C<sub>10</sub> to C<sub>20</sub> olefins or mixtures of i) and ii).

9. A fuel oil composition of claim 1, wherein the esters and/or amides of constituent B are derived from amines and/or alcohols having linear alkyl radicals.

10. A fuel oil composition of claim 8, wherein the comonomers B2) are esters of an acid selected from the group consisting of acrylic acid, methacrylic acid, maleic acid, fumaric acid, itaconic acid, and mixtures thereof with an alcohol selected from the group consisting of octanol, nonanol, decanol, undecanol, dodecanol, n-tridecanol, isotridecanol, tetradecanol, pentadecanol, hexadecanol and mixtures thereof.

11. A fuel oil composition of claim 1, wherein the comb polymer B has a molecular weight of between 1200 and 200 000 g/mol.

12. A fuel oil composition of claim 1, wherein the comonomers B2) are derived from  $\alpha$ -olefins having from 10 to 20 carbon atoms.

13. A fuel oil composition of claim 1, wherein a mixing ratio A:B is between 10:1 and 1:10.

14. A fuel oil composition of claim 1, further comprising polar nitrogen-containing paraffin dispersants.

15. A fuel oil composition of claim 1, wherein the proportion of F2 is greater than 2% by volume.

16. A fuel oil composition of claim 1, wherein the fuel oil of animal or vegetable origin comprises one or more esters composed of monocarboxylic acid having from 14 to 24 carbon atoms and alcohol having from 1 to 4 carbon atoms.

17. A fuel oil composition as claimed in claim 16, wherein the alcohol is methanol or ethanol.

18. A fuel oil composition of claim 1, wherein the fuel oil of animal or vegetable origin contains more than 4% by weight of esters of saturated fatty acids.

19. The fuel oil composition of claim 8, wherein the comonomers B2) are imides of an acid selected from the group consisting of maleic acid, fumaric acid, and itaconic acid, and mixtures thereof with an amine selected from the group consisting of octylamine, nonylamine, decylamine,

**19**

undecylamine, dodecylamine, tridecylamine, tetradecylamine, pentadecylamine, hexadecylamine and mixtures thereof.

**20.** The fuel oil composition of claim **8**, wherein the comonomers B2) are amides of an acid selected from the group consisting of acrylic acid, methacrylic acid, maleic

**20**

acid, fumaric acid, and itaconic acid, and mixtures thereof with an amine selected from the group consisting of octylamine, nonylamine, decylamine, undecylamine, dodecylamine, tridecylamine, tetradecylamine, pentadecylamine, hexadecylamine and mixtures thereof.

\* \* \* \* \*